

May 16, 1944.

B. BLUMENTHAL

2,348,719

PROCESS OF SEPARATING IMPURITIES FROM METALS OR ALLOYS

Filed Nov. 1, 1941



INVENTOR.

Bernhard Blumenthal  
BY

James K. Kent  
ATTORNEY

## UNITED STATES PATENT OFFICE

2,348,719

PROCESS OF SEPARATING IMPURITIES  
FROM METALS OR ALLOYS

Bernhard Blumenthal, Perth Amboy, N. J., assignor to American Smelting and Refining Company, New York, N. Y., a corporation of New Jersey

Application November 1, 1941, Serial No. 417,449

8 Claims. (Cl. 75—93)

This invention relates to the refining of metals and more particularly to a process of separating impurities from lead, tin and their alloys. The process is applicable for treating white metal, solder, type metal, terne, babbitt and similar bearing metals, as well as grid and coffin trimming metals.

Briefly, the invention resides in the discovery that relatively small amounts of impurities in metals and alloys can be economically and effectively removed by liquating the metal and simultaneously brushing or scraping the surface of the melt until tests indicate the impurities have been separated or their concentration lowered to the desired point.

In metallurgical refining processes, it has been conventional practice to employ drossing and skimming operations, for example, in softening lead bullion. The ordinary drossing and skimming operation, however, is not applicable for effecting the removal of impurities when present in very small amounts, for instance on the order of 0.01% or as low as 0.001%. Further, the usual drossing treatment is inadequate to accomplish separation of impurities from metals where there is very little difference between the specific gravity of the metal and the impurities. Similarly, the conventional drossing operation is inapt where the solubility limit of the substance to be separated is only slightly below or at the concentration to which the impurity is to be lowered. Further, removal of impurities by the customary drossing and skimming operations is ineffective where the impurities are suspended as suspensoids in the melt, or where various combinations of the aforementioned conditions are present. In all these cases it is impossible to remove the impurities by the ordinary skimming operation because there is no appreciable amount of skimmings formed which can be collected. Such operation merely stirs up the melt and disperses the impurities therein.

The process of this invention, however, overcomes these difficulties and provides a simple and highly efficient method of separating impurities, whether in the form of readily separable compounds or substances which are retained as suspensoids in the metal. This is the principal object of the present invention. Other objects and advantages of the invention will become apparent as the process is explained in detail.

For a more detailed description of my invention, the same is described in connection with a suitable form of apparatus useful for carrying out the improved process. Such an apparatus is

illustrated in the accompanying drawing and comprises a kettle 15, formed of suitable material, in which the metal to be refined is placed. Suitable means is provided for supporting the kettle 15, as shown at 16, and arrangement is made for heating the same as generally illustrated at 17.

A rotatable blade or paddle member 18 is mounted on the shaft 19 which is supported on the cross frame members 20 spanning the kettle. The motor reduction means 21 is drivingly connected to the shaft 19 and rotates the paddle at the desired R. P. M. Vertical adjustment of the paddle 18 on the shaft 19 is provided so that the paddle can be properly positioned with respect to the surface of the melt.

In operation, the metal to be refined is placed in the kettle and heated to form a melt as indicated at 22, and the paddle 18 is adjusted to dip very slightly into the metal bath. During liquation of the melt, the paddle is rotated. By repeatedly moving the paddle over the surface of the melt, metal is continually exposed to oxidation producing skimmings, which, as the paddle rotates, are brushed towards the sides of the kettle as shown at 23. As this operation continues the impurities migrate or float gradually to the surface and are wrapped up in the skimmings which are being continuously formed and scraped aside by the rotating paddle 18. Skimmings may be formed by other conventional methods with or without the formation of oxide skimmings. All that is required is that sufficient amount of skimmings be formed in which the substance or substances to be separated from the melt can be effectively gathered and removed.

The rotational speed of the paddle depends primarily on the surface area of the melt being treated and in each case is regulated so that the skimmings are not spattered out of the kettle, but merely pushed aside to expose fresh metal without appreciably stirring or agitating the body of the melt. In order to obtain the improved results, it is essential that the paddle be arranged to continually scrape aside the skimmings as they form while the metal is maintained unagitated and at such a temperature that the impurities or substances to be removed tend to separate out and move upwardly whereupon they come in contact with the skimmings and are mechanically occluded therewith. Preferably the temperature of the metal being treated is held within a narrow range such as will maintain the metal in a substantially liquid state and wherein the solubility of the substances to be

removed from the melt are at a minimum. The temperature usually is as low as possible, that is, just high enough to change the metal or alloy being treated from a solid to a liquid or partially liquid state. In each instance the physical conditions imposed on the melt are such as to create a tendency for the impurities, even though slight, to segregate from the base metal and contact the skimmings.

The following examples are given to show how effective my new process is in refining various kinds of metals and alloys. It will be understood, however, that the examples are merely typical and are not limitative of my invention.

#### Example 1

One hundred and fifty pounds of Linotype metal containing principally lead, with 12% antimony, 4% tin and having a sulphur content of 0.0016% was treated by my process at between 475° F. and 525° F. for approximately forty minutes. After removing the skimmings at the end of this time, it was found that the sulphur content was only 0.0005%. About 24 ounces of skimmings were formed or approximately 1% of the total weight of the melt. The surface area of the melt was about 32 square inches and the diameter of the area covered by the paddle approximated 7 inches. The paddle was rotated at 25 R. P. M.

A conventional practice of removing sulphur from white metals comprises the introduction of caustic soda or the like alkaline earth compound. The process of this invention eliminates the necessity of adding substances to effect the removal of small amounts of sulphur, and produces a metal which is substantially free from impurities. Further, the total weight of the skimmings produced during the process is much less than in the case of ordinary drossing and skimming operations. This lowers the cost of the refining operation.

#### Example 2

One pound and ten ounces of Linotype metal, of similar composition as Example 1 but containing 0.0056% sulphur, was treated in a small research laboratory apparatus, comparable to that illustrated in the accompanying drawing, for ten minutes and while heated to about 540° F. The surface area of the melt was approximately 10 square inch and the paddle was rotated at 100 R. P. M. The area scraped by the paddle had an approximate diameter of about 2 inches. After removal of the skimmings, the resultant metal analyzed only 0.0002% sulphur. One-half ounce of skimmings was formed constituting about 2% of the melt.

#### Example 3

A similar weight of Linotype metal, as in Example 2, containing 0.011% aluminum was treated at 540° F. as described. In this case the aluminum was entirely removed.

In the usual practice, the last traces of aluminum in type metals are removed by treating the metal, either with metallic alkalies or with molten alkaline salts using cobinations of caustic soda, sodium carbonate, or alkali chlorides. My process, however, avoids the use of addition compounds and provides a more effective and less costly method of separating aluminum.

#### Example 4

A like quantity of Linotype metal as in Example

2 was treated as therein described. In this instance the type metal contained 0.01% zinc which had been previously partially removed as zinc sulphide by treatment with sulphur. When the sulphur treated metal was heated to 550° F. and scraped for ten minutes, in accordance with my process, it was found that both the zinc and sulphur were removed.

In the ordinary practice, zinc is separated from type metals by treating the metal with air or steam. This produces a large amount of dross and involves the loss of tin. Since zinc considerably increases the rate of drossing of type metals, when present, it is necessary to remove it completely, and my process provides a simple and improved method for doing this.

#### Example 5

A solder comprising approximately 60% lead and 40% tin, and containing 0.016% nickel, was treated as described in Example 2. After treatment, the nickel content was found to have been lowered to 0.008%.

In the customary kettle operations it is difficult to remove small amounts of nickel, whereas as by employing the process of this invention it is easy to produce metal having less than 0.01% nickel. This is a decided improvement over the results attained by prior methods of refining.

#### Example 6

Linotype metal containing 0.06% tellurium was treated by my process, as described in Example 2, at a temperature of approximately 540° F. The refined type metal was found to have only 0.01% tellurium after scraping the melt for ten minutes during liquation of the metal.

In light of the above test results it will be evident I have devised a singularly simple and efficient method for treating metals and alloys to remove impurities which does not require the addition of costly reagents. Furthermore, my new process can be carried out with inexpensive equipment and is more easily performed than the intricate processes used prior to my discovery. While I have described my process in detail with respect to certain metals and alloys, it will be understood that the process is applicable broadly to metallurgical refining processes and that various changes may be made within the scope of the invention as defined by the appended claims.

What is claimed is:

1. The process of refining metals or alloys of the group consisting of lead and tin to remove impurities which are present in amounts not greatly in excess of the amount which is soluble in a melt formed of the impure metal being refined and will float to the surface of said melt comprising the steps of liquating the metal at a substantially constant temperature wherein the impurities tend to segregate from the melt and approach the surface thereof, simultaneously skimming the surface of the melt in a continuous manner without appreciably disturbing the body of the melt to scrape aside the skimmings and expose fresh metal for oxidation, and continuing the operation at said temperature until the impurities have been lowered to the desired point.

2. In the process of refining lead and tin metals or alloys to remove impurities which are present in amounts not greatly in excess of the amount which is soluble in a melt formed of the impure metal being refined and which insoluble impurities will float or migrate to the surface of said melt, the steps of heating the metal in an oxidiz-

ing atmosphere to a temperature at which the solubility of the impurities in the melt is at a minimum, skimming the surface of the melt continuously while maintaining said temperature substantially constant for a predetermined length of time to remove substantially all of said insoluble impurities, said skimming operation being performed without substantially agitating or stirring the body of the melt to effect mechanical occlusion of the impurities in the skimmings as they segregate from the metal and rise to the surface of the melt.

3. The process of removing small amounts of impurities from type metals wherein said impurities are present in amounts not greatly in excess of the amounts which are soluble in a melt formed of the impure metal and which impurities will float to the surface of said melt comprising heating the metal while exposed to air to substantially its liquid state, holding the metal at this temperature, simultaneously and continuously scraping at least a portion of the melt surface to repeatedly expose fresh metal to oxidation without appreciably disturbing the body of the melt forming skimmings which are continually brushed aside, continuing the operation to effect occlusion of the impurities in the skimmings until the content of said impurities in the melt has been lowered substantially to an amount below which the impurities are soluble in said melt.

4. The process of removing small amounts of sulphur from metals or alloys of the group consisting of lead and tin wherein said sulphur is present in an amount not greatly in excess of the amount which is soluble in a melt formed of the impure metal and floats to the surface of said melt comprising heating the metal until it is substantially in a liquid state, holding the temperature at this point while maintaining said liquid metal in an oxidizing atmosphere to form oxide skimmings on the surface of the melt, simultaneously scraping at least a portion of the surface of the melt to scrape the skimmings aside without stirring the body of the melt, continuing the scraping operation while maintaining the melt at said temperature to mechanically collect the sulphur or compounds thereof in the skimmings, and removing the same therewith.

5. The process of removing residual impurities from lead and tin base solder metal wherein said impurities are present in amounts not greatly in excess of the amount which is soluble in a melt formed of the impure metal and rise to the surface of said melt which comprises heating the metal until it is substantially in a liquid state, holding the temperature at this point while maintaining said liquid metal in an oxidizing atmosphere to form oxide skimmings on the surface of the melt, simultaneously scraping at least a portion of the surface of the melt to scrape the skimmings aside, continuing the scraping operation while maintaining the body of the melt in a quiescent state to mechanically collect the impurities or compounds thereof in the skimmings, and removing the same therewith.

6. The process of removing impurities from metals or alloys of the group consisting of lead and tin when present in small percentage amounts of the order of 0.01% or in amounts not greatly in excess of the amount which is soluble in a melt formed of the impure metal being refined and will float to the surface of said melt comprising heating the metal in a receptacle while exposed to oxidation by surrounding air to a temperature wherein liquation of the melt occurs, maintaining said melt at this temperature while concurrently lightly skimming the surface of the melt to scrape aside the skimmings and repeatedly expose fresh metal to the air without disturbing the body of said melt and continuing said treatment to effect the mechanical occlusion of the impurities in the skimmings as said impurities migrate to the surface of the melt whereby the same can be removed with said skimmings to reduce the content of impurities to the desired minimum.

7. The process of removing impurities from lead and tin metals or alloys thereof wherein said impurities are present in amounts not greatly in excess of the amounts which are soluble in a melt formed of the metal and containing said impurities which impurities float or migrate to the surface of the melt comprising heating the metal to produce a melt, maintaining the melt in an oxidizing atmosphere to form oxide skimmings on the surface of the melt, simultaneously skimming the surface of the melt in a continuous manner scraping aside the skimmings while the body of the melt remains in a quiescent state whereby the insoluble impurities which rise to the surface of the melt are mechanically occluded in the skimmings and scraped aside therewith and continuing said treatment until the content of said impurities in the melt has been substantially lowered or reduced to a value below which amount the impurities are soluble in the melt.

8. The process of removing impurities from lead and tin metals or alloys thereof wherein said impurities are present in amounts not greatly in excess of the amounts which are soluble in a melt formed of the metal and containing said impurities which impurities will float or migrate to the surface of said melt comprising establishing a melt of the impure metal, maintaining the melt in an oxidizing atmosphere to form oxide skimmings on the surface of the melt, skimming the melt in a continuous manner without stirring the body of the melt whereby the insoluble impurities as they rise to the surface of the melt are mechanically occluded in the skimmings and subsequently removed therewith and continuing the simultaneous oxidation and skimming operation to effect the mechanical occlusion of said impurities in the skimmings as they rise to the surface of the melt until the content of said impurities in the melt has been substantially lowered or reduced to an amount below which the impurities are soluble in the melt.